

Jan. 13, 1970

M. A. LEVINSTEIN

3,489,534

LIGHTWEIGHT METALLIC STRUCTURE

Filed Jan. 3, 1967



INVENTOR  
MOSES A. LEVINSTEIN  
BY  
*Lee R. Fuchs*  
ATTORNEY —

1

3,489,534

### LIGHTWEIGHT METALLIC STRUCTURE

Moses A. Levinstein, Cincinnati, Ohio, assignor to General Electric Company, a corporation of New York  
Filed Jan. 3, 1967, Ser. No. 606,943  
Int. Cl. B23k 31/00; B21f 45/00; B21c 37/00  
U.S. Cl. 29—191.6

6 Claims

#### ABSTRACT OF THE DISCLOSURE

A lightweight metallic structure, such as a shroud, includes hollow wires bonded together. The wires are an alloy including at least one of aluminum, magnesium or their alloys and at least one of iron, nickel, cobalt or their alloys.

This invention relates to lightweight metallic structures and, more particularly to such a structure including members such as filaments, strands or wires of metal bonded together.

Lightweight mesh, fabric or metal wool structures, hereafter called mesh, employing strands, wires or filaments, hereafter called wires, held to or bonded with one another, alone or as a support for other members, use such wires in solid form in uniform or random arrangements. Such wires can be bonded together by welding, brazing and the like.

One use for such a structure is as a gas seal held between successive stages of an axial flow turbine. In such an application layers of mesh bonded to holding members, are located opposite the tips of blading members. In some applications filler materials are disposed between wires. Because of the variety of metals available for the wires and variety of available filler or bonding material, abrasibility, temperature resistance, oxidation resistance and the like can be selected for the mesh. However, because commercially available fine wires are solid, the density of the material is greater than that which would be most desirable, particularly for use in an aircraft gas turbine where weight is an important factor.

It is the principal object of the present invention to provide an improved lightweight metallic structure including layers of fine hollow wires or mesh to decrease the density of the structure.

Another object is to provide an improved, lightweight gas turbine abradable shroud.

These and other objects and advantages will be more clearly understood from the following detailed description, examples and the drawing.

In the drawing:

FIG. 1 is a sectional isometric view of a wire having a solid metallic core and a continuous metallic shell prior to processing;

FIG. 2 is a sectional isometric view of the wire of FIG. 1 after processing;

FIG. 3 is a partially sectional isometric view of a shroud including the structure of the present invention;

FIG. 4 is a more detailed sectional view of a shroud of the present invention including stacked unwoven wires; and

FIG. 5 is a sectional view of the upper portion of the shroud as shown in FIG. 4 with wires in the form of a mesh.

In order to attain and fulfill the above objects, a lightweight metallic structure is made by providing a metallic wire or mesh core of a first metal and then coating it, such as by electro or vapor deposition, with a shell of a second metal to produce a composite wire or mesh. The crystal relationship and relative diffusion rates between the core metal and the shell metal is such that the core metal will diffuse preferentially into the shell metal to

2

produce a wire or mesh having a hollow interior bounded by the shell metal. This will occur when the composite wire or mesh is heated at a temperature below the melting point of the shell metal and in the absence of a shell-crushing pressure. Metals which can be used in this manner for a core material include aluminum, magnesium and their alloys. Metals which can be used as the coating or shell material include iron, nickel, cobalt and their alloys.

According to one form of the present invention, after 10 a core wire is coated, the composite wire thus formed can be arranged into a mesh or other desired configuration. A plurality of meshes or individual wires can be stacked beside or one upon the other or both to provide whatever thickness is desired. Then the composite members are held 15 in intimate contact at various points along their surfaces and heated at that temperature sufficient to diffuse the core metal into the shell metal but below the melting point of the shell metal. The result is a lightweight porous structure comprising a plurality of wires or meshes bonded one to the other, each wire or mesh having a hollow core. 20 If more rigidity, ductility, bonding or body is desired, solid wires or powdered filler material such as brazing alloys or both can be intermixed or interwoven with the composite wires or meshes.

Described in co-pending application Ser. No. 606,963, filed Jan. 3, 1967 and assigned to the same assignee as this invention is a method for making hollow members which includes the making of hollow wires, meshes and tubes. It has been found that if, during heating to diffuse 30 the core metal into the shell metal, a plurality of composite wires or meshes are maintained in contact under sufficient pressure to maintain the contact but not sufficient to cause collapse of walls of the hollow wires produced, the wires not only can be made hollow but also can be bonded into a more rigid structure.

Referring to the drawing, the isometric sectional view of FIG. 1 shows a composite wire 10 having a core 11 most conveniently and preferably of a metal of the group aluminum, magnesium and their alloys. Surrounding the core is a coating or shell 12 of a metal into which core 11 will diffuse upon heating to a temperature such as above the melting point of core 11. Most desirable shell metals for this purpose are metals of the group of iron, cobalt, nickel and their alloys.

45 After heat treatment according to the present invention, such as about an hour at 2000° F., core 11 of the composite wire 10 in FIG. 1 diffuses into shell 12 to form an alloy 14 as shown in FIG. 2. When such a metal as aluminum is used for the core and nickel for the shell, it has been found that original composite wire outside 50 diameter  $d$  in FIG. 1 increases to hollow wire outside diameter  $D$  in FIG. 2. If a plurality of stacked mesh including composite wires is contained in a fixed volume during heat treatment, such increase in diameter produces a slight pressure between the wires. This assists in bonding together during processing the plurality of composite wires. Therefore, a holding or confining structure in which the plurality of wires or meshes are placed can be shaped 55 to provide a desired arrangement.

60 One such arrangement which can be made is shown in FIG. 3 during the practice of the method of this invention. A sectional view of the product is shown in FIG. 4. Referring to those two figures, a shroud backing member 16 of a stator portion of an axial flow turbine, for use 65 opposite rotating blades, was placed on a fixture base 18 having a curved surface 20 adapted to receive the shroud member. A nickel base brazing alloy powder 22, in the form of a paste or slurry, was placed on the exposed surface of shroud member 16. Solid wires of a nickel base alloy 24, sometimes referred to as Nichrome alloy, were placed over the brazing alloy 22. In another example substantially pure nickel wire mesh was used.

Composite wires 26 made of 15-40 mil aluminum wire as the core with a 5-10 mil thick coating of nickel as the shell were then placed on the solid wires 24. By weight, this consisted of 20-27% Al and 73-80% Ni. As shown in FIG. 5, the wires can be partially or entirely woven together into a mesh. A top holding plate 28 was placed on the stacked wire-brazing alloy combination. In order to assure bonding of the various wires and brazing alloys together and to the shroud backing member 16, a slight holding pressure, represented by arrow 30, was applied to the stacked wires through holding plate 28. For example, this can be accomplished by clamping strips or other clamping means well known in the art. However, the pressure applied should be less than that which would cause collapse of the hollow wire during or after processing.

The clamped structure was then heated for one hour at about 2000° F. in argon to diffuse the aluminum core 11 into shell 12 to form a shell 14 of a nickel-aluminum alloy as shown in FIGS. 1 and 2. This produced hollow wires 26 of FIG. 4 or FIG. 5. At the same time, the heat treatment bonded wires 26 together and to wire mesh or structure 24 and also brazed solid wires 24 to shroud 16 to form the abradable shroud shown in FIG. 4.

In another specific example, 25 mil aluminum wires were first coated with 7.5 mils of nickel by electroplating. The nickel-aluminum alloy 14 in FIG. 2 was produced after diffusion of the aluminum wire into the nickel shell in an argon atmosphere furnace in which the temperature was increased over a period of about 2 hours from room temperature to 2000° F. The material was then held for 1/2 hour at 2000° F. after which it was slowly cooled over a period of about 1 hour. The relatively slow heat up period or rate is desirable to avoid rupture of the shell wall as a result of too rapid a diffusion and expansion. However, frequently in the manufacture of shrouds as described above, some incidence of shell wall rupture in the tubular structure can be tolerated: the density is not appreciably increased and the high porosity and void space through a very high percentage of the remainder of the tubes and structure provides the material with suitable abradability.

In one example, a 99% aluminum core in the form of a 120 x 120 mesh of 4 mil wire in a twill weave first was coated as a unit with 1.5 mils of nickel in an electroplating bath. Such coating by electroplating or vapor deposition can be accomplished readily with well known processes having sufficient throwing power to deposit nickel over virtually the entire exposed surface. By moving the electroplating holder from time to time during plating, a substantially completely coated composites structure can be produced. Then upon heating to diffuse the core into the shell, some thin walls or even ruptures may result at or near the points of contact between wires of the core mesh. However, as was mentioned above, this is not necessarily important in an abradable shroud of the type described above. In some cases, there are no breaks at such points of contact. If any breakthrough in the wall

structure of the final hollow tubular member is to be specifically avoided, then the core wires should be coated individually prior to their being woven or grouped into a mesh, fabric, metal wool and the like.

It has been found that composite wires having a core consisting essentially of 5-35 weight percent of the composite wire are preferred for use in the present invention. Below about 5%, too small a void is created because of expansion of the wire during processing. A core greater than about 35 weight percent results in too thin a shell.

Although description of the present invention has included specific examples and embodiments, these are meant to be typical of the invention rather than any limitation. It is intended by the appended claims to cover the various modifications and variations of which the invention is capable within the knowledge of one skilled in the art.

What is claimed is:

1. An improved lightweight metallic structure comprising:

a plurality of hollow wires bonded together; the hollow wires being an alloy of at least one element selected from the group consisting of Al, Mg and their alloys and at least one element selected from the group consisting of Fe, Ni, Co and their alloys; the structure having a thickness of a plurality of hollow wires.

2. The structure of claim 1 in which a plurality of solid wire members are bonded with the hollow wires.

3. The structure of claim 2 in which there is at least one layer of wires in the form of a mesh.

4. An improved lightweight shroud comprising:

a backing member; and a plurality of layers of hollow wires bonded together into the backing member; the hollow wires being an alloy of at least one element selected from the group consisting of Al, Mg and their alloys and at least one element selected from the group consisting of Fe, Ni, Co and their alloys.

5. The shroud of claim 4 in which a plurality of solid wire members are bonded with the hollow wires.

6. The shroud of claim 5 in which at least one of the layers of wires is in the form of a mesh.

#### References Cited

##### UNITED STATES PATENTS

|           |        |          |       |          |
|-----------|--------|----------|-------|----------|
| 2,271,662 | 2/1942 | Rubisow  | ----- | 210—169  |
| 3,087,233 | 4/1963 | Turnbull | ----- | 29—182   |
| 3,123,446 | 3/1964 | Wheeler  | ----- | 29—183   |
| 3,266,130 | 8/1966 | Glaze    | ----- | 29—163.5 |

L. DEWAYNE RUTLEDGE, Primary Examiner

E. L. WEISE, Assistant Examiner

U.S. Cl. X.R.

29—193, 471,1